

## UNITED STATES PATENT OFFICE

2,479,037

## STENCIL DUPLICATING INKS

Thomas Seal Chambers and Robert Thompson  
Florence, Chicago, Ill., assignors to A. B. Dick  
Company, Chicago, Ill., a corporation of Illinois

No Drawing. Application September 18, 1948,  
Serial No. 49,994

19 Claims. (Cl. 106—26)

1

This invention relates to ink compositions and especially to stencil duplicating inks for use with rotary stencil duplicating machines or for other stencilling operations wherein ink is transferred through a stencil to an impression medium.

Stencil duplicating inks are unlike other inks in the sense that certain physical characteristics are demanded of the ink to function properly in the duplicating machine to produce copy quality of uniform and acceptable character. Functionally, the ink is supplied in continuous fashion to an ink pad, other like reservoir or distributing medium, and after uniform distribution therein, it is transmitted through the stencil openings to the impression medium chiefly by forces developed at the point of contact between the rotating cylinder and the impression roller. Drying generally occurs by absorption of the vehicle or carrier into the pores or interstices between the fibers of the paper. Some of the characteristics by which stencil duplicating inks are distinguished are set forth below:

1. Sufficient flow of a desired character is necessary to enable the ink to distribute itself quickly and uniformly throughout the ink pad and to effect satisfactory transmission through the stencil to the impression medium. Not so much flow is demanded as will cause the ink to drip or run from the ink pad or to flood the stencil, whereby undesirable copy is obtained. In the event that the flow is insufficient, ink distribution in the pad and transmission through the stencil are such as to produce copy of variable and undesirable characteristics. Viscosity is used as a measure of certain flow characteristics. Yet, we find it impractical presently to define the desired flow characteristics of inks rigidly and exclusively in the terms of viscosity. The optimum viscosity values vary widely according to the materials of which the ink is formulated and the instrument by which the measurements are made.

2. The ink composition should be quick drying when applied to impression paper; otherwise, it would be necessary to resort to special devices and costly practices in order to handle the copy within a reasonable time and eliminate setoff. The commonest device to cope with this problem is the practice of slipsheeting; that is, inserting interlayer sheets between successive copies as they are duplicated. The problem may be alleviated to a limited extent by using as the impression medium highly absorbent paper which rapidly distributes the vehicle but makes it practically impossible to obtain sharply defined copy because of "feathering" of the ink.

3. The drying characteristics should not be such as to cause premature hardening of the ink on the pad or clogging of the stencil openings. These objectionable features which ordinarily

2

cause poor copy are minimized or substantially prevented by the use of relatively slow drying inks. Slow drying inks remain in such condition that ink removal from the stencil, ink pad, or machine parts may be effected in a simple manner. The combination of characteristics calling for quick drying on the impression medium, on the one hand, and slow drying on the pad, on the other hand, is difficult to achieve.

4. A suitable ink should be sufficiently stable to minimize, or even eliminate, inadvertent separation of ingredients, prior to use or while in use, such as might lead to operating difficulties. The tendency of pigments to rearrange themselves in non-uniform distribution and the tendency of emulsions, when used, to break are constant sources of such operating difficulties, causing clogging of the ink pad, stencil or cylinder, and making it practically impossible to obtain copy of acceptable quality.

5. An ink composition for use with stencil duplicating machines should be non-corrosive to the machine parts. It should be safe to handle, easy to manufacture, and have good shelf life.

6. The ink should not give "show-through"; that is, there should be little visibility of the copy from the opposite side of the impression paper. It should not give an oily or colored outline or "halo."

7. It is desirable, when possible, to have an ink which, after transfer to the impression medium, is relatively resistant to moisture, and a wide variety of solvents, greases, chemicals, and the like. It should be resistant, therefore, to wetting, perspiration developed by the hands, and various organic and inorganic materials present in processes, products, and apparatus with which duplicated material might come in contact.

Ink compositions capable of meeting the majority of these characteristics have been the subject of considerable research since the advent of stencil duplicating machines in the latter part of the nineteenth century. Actually, little change has taken place in stencil duplicating ink formulations over and above those initially developed. The earlier stencil duplicating inks were pigmented oil-base compositions containing as much as 80 percent and sometimes 90 percent oil, which were mostly non-drying oils, such as castor oil, coconut oil, and the like. Often a binder, such as rosin, was incorporated to improve the viscosity and other characteristics of the ink. In order to effect solution of the binder, a solubilizing agent, such as a rosin oil, was often incorporated. These inks were burdened by the fact that the presence of the oils, and especially the non-drying oils, which functioned as the carrier or vehicle for the pigments, caused a highly objectional degree of setoff and smear, unless special devices were used in handling the impression medium.

In addition, the high percentage of oils was directly responsible for the objectionable oily letter outline or "halo" in copy prepared with the ink. From the standpoint of economics, past experience has shown that natural fats and oils are frequently and unpredictably in short supply, and this impairs suitable standardization or economical formulation of oil-base inks.

In attempting to improve oil-base inks, emulsion inks were subsequently developed. Stencil duplicating inks of the oil emulsion type very often contained less oil to relieve some of the described objectional features of oil-base inks but new problems were presented which inhibited their utility in actual practice. The emulsion inks presented an operating problem because they often separated before or while in use, whereby the ink pad or the stencil or both became clogged to prevent uniform distribution of the ink and complicated the production of good copy. In addition, the inner phase of the emulsion frequently contained sulfonated glycerides which were corrosive to elements and machine parts associated therewith.

It is an object of this invention to produce a stencil duplicating ink which overcomes the objectionable features of prior inks and meets substantially all of the desirable characteristics of a good stencil duplicating ink.

Another object is to produce a stencil duplicating ink constituted primarily with miscible ingredients to minimize the danger of separation which might impair the quality of the ink or its function in the duplicating machine.

A further object is to produce a stencil duplicating ink which is substantially free of oils whereby fast drying and good copy are obtained without the objectionable features of "show-through" and "halo."

A still further object is to produce a stencil duplicating ink which may be used with relatively non-absorbent paper stock or with hard and highly finished surfaces on the impression medium, materials which were incapable of use with prior stencil duplicating inks.

Another object is to produce an ink of the type described which is quick drying to enable handling almost immediately after duplicating without fear of setoff or smearing and which, after drying, becomes insolubilized to water to the extent that it is unaffected by moisture, high humidity, solvents, greases, oils, hydrocarbons, and the like.

Another object is to produce a stencil duplicating ink which is substantially non-corrosive, and simple, easy, and safe to manufacture and handle.

An object of this invention is to produce a water-base stencil duplicating ink wherein water comprises the principal diluent and carrier and is combined with other substances adapted to impart color, body, penetrability, drying, and insolubility characteristics desired in a stencil duplicating ink.

These objects are accomplished according to our invention by formulating a water-base stencil duplicating ink in which water comprises the major diluent and functions primarily as the carrier or vehicle for the tinctorial matter. The desired body and flow of the desired character is derived from the use of a cellulose derivative which is miscible with the diluent to form a stable, non-corrosive solution that is safe to handle and easy to manufacture. The cellulose derivative not only imparts bodying character-

istics to the composition but also functions as an adherent base upon drying to permit duplicating on non-absorbent and highly finished paper stock. When desired, a water-soluble reactant may be incorporated to insolubilize the resin or bodying agent when transferred to the impression medium.

As the tinctorial agent, use may be made of water soluble dyes, such as nigrosine dye of the type Nigrosine WSJ. Use may also be made of other water soluble acid and basic dyes, such as triphenylmethane, rhodamine, thioflavine, and auramine dyes, or sulfonated triphenylmethane, quinone-imide and xanthone dyes. Representative of the acid dyes which have been successfully used are the materials marketed by Calco Chemical, a Division of American Cyanamide Company, under the trade name "Calcocids," which include the mono-, di-, and tri-sodium sulphonate derivatives of the nitro, azo, pyrazoline, quinoline, triphenyl-methyl, diphenyl-naphthylmethane, azine, xanthone and anthrone groups. To a limited extent, the azo dyes may also be incorporated as the tinctorial agent in ink formulations of the type described. Instead of dye compounds, dispersions of inorganic pigment may be used in which the pigments may comprise carbon black, lamp black, malachite green, iron blue, cadmium yellow, and the like. The amount of dye in the ink formulation depends on the chemical nature of the coloring material used. Some dyes are capable of imparting sufficient color to lend legibility to the copy when little is used, while with others, it is necessary to use higher concentrations of dye to secure the desired effect. The lower limit of the dye concentration, therefore, is determined by its tinctorial strength which varies widely from compound to compound. The upper limit often is influenced by solubility factors or by the effect of the dye on other ingredients of the ink composition, as, for example, in causing gelation of the resinous material. We have found that 3 to 7 percent Nigrosine WSJ is suitable for these water-base inks. The amounts of other dyes may be more or less according to their characteristics, as pointed out above. When pigments are used, it is often desirable to use concentrations ranging from 3 to 15 percent or more of the ink composition when calculated on a weight basis.

By the phrase "cellulose derivative miscible with water" it is meant to include cellulose ethers soluble in water or dilute aqueous alkaline solutions, such as the hydroxylated cellulose ethers in which there are sufficient hydroxyl groups to influence solubility in aqueous medium. Among the water soluble ethers of cellulose which find excellent use in stencil duplicating ink formulations of the type described are the hydroxylalkyl celluloses, such as hydroxyethyl cellulose. Use may also be made of the partially alkylated cellulose ethers, such as a medium viscosity methyl cellulose or ethyl cellulose having less than 19 percent ethoxy groups. We have found that the water soluble salts of carboxy methyl cellulose, such as sodium or ammonium carboxy methyl cellulose, may also be used. The amount of water soluble cellulose ether derivative required to impart the desired flow characteristics varies according to the degree of polymerization or the average molecular weight of the cellulose ether derivative, the degree of alkylation, the groups of which the cellulose ether is constituted, and to a lesser extent according to the substances by which the resinous materials are taken into solution. In

actual practice, sufficient body in the ink composition is derived for use with present duplicating machines when the composition contains 2 to 10 percent hydroxyethyl cellulose (Cellosize), but more or less may be used when desired. Since the bodying capacity of suitable resinous materials varies according to their molecular construction, it is more expedient to define the limitations as to the amounts of bodying agents in accordance with their resulting influence on flow characteristics. This can be determined by ordinary viscosimeters as the measurement corresponding to a viscosity of about 35 to 150 seconds measured by a Stormer viscosimeter operating with a standard cup without a center baffle at 20° C. under a 200 gram load. Of course, it will be understood that as the requirements of duplicating machines change in the course of developments in the art, the viscosity limitations and, therefore, the amount of bodying agent may change accordingly without departing from the invention.

A valuable feature of this invention resides in the fact that the water soluble cellulose ethers of the type described are constituted with hydroxyl groups capable of reaction with an aldehyde to insolubilize the resinous material. Similarity exists between the possible reaction and that of the acetal reaction between carbonyl and hydroxyl groups. When use is made of an aldehydic substance capable of latent reaction to insolubilize the resinous material upon drying, excellent stability and shelf life of the ink composition are secured before duplication, and after transfer to the impression medium, the desirable characteristics of quick drying and resistance to moisture, and many solvents, greases, oils, hydrocarbons, and the like are secured. One such latent aldehydic substance is glyoxal and another, less reactive and consequently used in greater amounts, is pyruvic aldehyde. Either of these substances may be referred to as bifunctional carbonyl compounds, which, in the presence of catalyst or upon drying, are capable of the acetal reaction. Each has at least one functional aldehyde group. Insolubility may result from the elimination of hydroxyl groups, the formation of hemi-acetals, or the cross linking of cellulose molecules, as is typical of the acetals. Insolubilization may also be derived, even in the absence of glyoxal, from the loss of ammonia in the event that an ammonium salt of a carboxy cellulose ether is used. 0.25 to 3.0 percent of glyoxal based upon the weight of the ink composition is usually sufficient, and as much as 7 percent has been used, but best results are secured when the cellulose resin and aldehyde are present in the ratio of about 2 to 10 parts by weight of the resin to 1 part of the aldehyde.

In order to increase the penetrability into the impression paper and in order to improve the characteristics of the ink with respect to distribution through the ink pad and stencil, a wetting agent may be added to the composition. A suitable wetting agent may be selected from the group consisting of the diethyl esters of sodium sulfosuccinate (Aerosols), quaternary ammonium salts (Tritons), substituted aromatic sulfonates (Duponols), dibutylphenol sodium disulfonates (Areskelene), sulfonated ethers (Tensol), and the like. Less than two percent of the wetting agent ordinarily is sufficient to impart the desired wetting characteristic, although more may be used when desired.

In order to minimize the tendency of the inks

5 to dry too rapidly before transfer to the impression medium even under conditions of high temperature or low humidity, in order to provide an adherent base after the water has been removed which is flexible and has desirable physical characteristics, and to improve wet strength and moisture resistance, a non-volatile organic liquid compatible with the solution of the water soluble cellulose ether is added. These properties are derived by the addition of polyhydric alcohols, such as glycerine, ethylene glycol, diethylene glycol, polyglycols, and the like. An important and most beneficial phenomenon is derived from the use of polyhydric alcohols in ink formulations of the type described. Polyhydric alcohols in proper amounts appear to increase the stiffness, that is impart a false body to the ink to the extent that free flow is apparently reduced. By their use, ink leakage from the cylinder or inadvertent flow of the ink composition from the pad or stencil is noticeably reduced. Actually, the apparent increased stiffness is not measurable by a viscosimeter operating at high rates of shear. As a result, it is not apparent upon transfer of the ink to the impression medium because flow under high shearing rates results when the ink is forced through the stencil. The polyhydric alcohols may react with the aldehyde conjointly with the cellulose ether derivative to form acetals and cross-linkages. In specific applications, amounts ranging from 1 to 25 percent by weight of ethylene glycol have been successfully used with compositions constituted with hydroxyethyl cellulose of medium viscosity as the bodying agent. When more is used, there is a tendency to disturb the colloidal state of the ingredients of the ink composition. Corresponding amounts of other polyhydric alcohols may be used. The upper limit of concentration of any selected polyhydric alcohol or combination of polyhydric alcohols with the same or other types of suitable cellulose ethers is that which causes gelling or other undesirable disturbance of the colloidal state of the system.

45 The following examples will illustrate water-base stencil duplicating inks embodying features of our invention:

#### Example I

| Percentage | Material                                                       |
|------------|----------------------------------------------------------------|
| 77.5       | Water.                                                         |
| 5.0        | Nigrosine WSJ (water soluble dye).                             |
| 6.0        | Hydroxyethyl cellulose (100 c. p. s. in 10% aqueous solution). |
| 1.0        | Aerosol OT.                                                    |
| 10.0       | Ethylene glycol.                                               |
| 0.5        | Glyoxal.                                                       |
| 100.0      |                                                                |

#### Example II

| Percentage | Material                                       |
|------------|------------------------------------------------|
| 69.2       | Water.                                         |
| 15.0       | Aquablack M (40% aqueous carbon black slurry). |
| 1.8        | Methyl cellulose (400 c. p. s.)                |
| 1.0        | Aerosol OT.                                    |
| 10.0       | Diethylene glycol.                             |
| 3.0        | Pyruvic aldehyde.                              |

70 Glyoxal and pyruvic aldehyde are normally incorporated as a 30 percent water solution; however, the amounts designated in the above examples refer to the dry weight of the free aldehyde. While the materials may be combined in any order since they are generally miscible

one with the other, it is usually preferred to prepare the solution of resin in the liquid vehicle first. The above formulations have a viscosity within the range of 50-100 seconds, as measured by a Stormer viscosimeter of the type previously described. By comparison, viscosities of suitable oil base stencil duplicating inks may be about 400-500 seconds and many suitable oil base emulsion inks may have viscosities of about 250-350 seconds.

When water insolubility is unimportant, the bifunctional carbonyl compound may be omitted. In the event that the insolubilizing agent is omitted, the ink is not entirely devoid of moisture resistance because the polyhydric alcohols function, to an extent, as a protective agent for the inks and they impart some degree of water resistance.

By the use of our new and improved stencil duplicating ink, drying takes place at a speed which is beyond that heretofore contemplated for stencil duplicating inks, making it possible to handle the copy immediately. It is possible to eliminate setoff without the costly and cumbersome technique of slipsheeting. It is possible to duplicate on hard stocks and highly finished impression media and still handle the work immediately. The ink produced by this invention dries rapidly on bond, ledger, card, or enamel stock, papers which have heretofore not been suitable for widespread use with stencil duplicating machines.

There are no materials present in such quantity to cause undesirable "show through" or "halo." This is because the present carrier and diluent is water which may be completely eliminated from the impression medium and is not resident as are the oils of prior duplicating inks.

It will be evident that other important advantages are derived from the use of water-base stencil inks including the elimination of possible separation of the ink in use or prior to use because the ink composition is stable; simplification in the processes of cleaning the machine and stencil by the use of a simple water rinse as effected by a dip or spray because the ink composition before transfer to the impression medium is readily soluble in water and many of the common solvents; self-sealing characteristics derived from the use of the polyhydric alcohol and cellulose ether derivative to reduce the tendency of the inks to drip inadvertently or leak from the container or cylinder because of the high body of the ink composition in the free state; simplicity in ink manufacture because preparation is effected by solution which eliminates grinding or other tedious means for incorporating the colors and resinous material.

It will be understood that the basic substances may be prepared for marketing in concentrated or dry form to be diluted at the station of use with water before filling the ink container. It will further be understood that other miscible solvents may be partially substituted for the water as the diluent or diluting substance, such, for example, as the lower alcohols and the like. In addition, it will be understood that numerous substitutions may be made in the materials and their amounts without departing from the spirit of the invention, especially as defined in the following claims.

We claim as our invention:

1. A stencil duplicating ink comprising an aqueous composition consisting essentially of water as the diluent, a tinctorial agent to impart

legibility to the copy, a water soluble cellulose derivative selected from the group consisting of cellulose ethers and cellulose esters having water solubilizing hydroxyl groups and a latent aldehyde selected from the group consisting of glyoxal and pyruvic aldehyde.

2. A stencil duplicating ink comprising an aqueous composition consisting essentially of water as the diluent, a tinctorial agent, a water soluble cellulose ether for bodying the composition and for operating as an adherent base upon drying, a liquid polyhydroxy alcohol compatible with the solution of cellulose ether in diluent, and a wetting agent.

15 3. A stencil duplicating ink comprising an aqueous composition consisting essentially of water as the diluent, a tinctorial agent, a water soluble cellulose ether for bodying the composition and for operating as an adherent base upon drying, a liquid polyhydroxy alcohol compatible with the solution of cellulose ether in diluent, a wetting agent, and an aldehyde selected from the group consisting of glyoxal and pyruvic aldehyde.

4. A stencil duplicating ink comprising more

25 than 50 percent water as the diluent, from 3 to 15 percent of a tinctorial agent, from 1 to 25 percent of a water soluble hydroxylated cellulose ether, from 1 to 25 percent of a liquid polyhydroxy alcohol compatible with the solution of the cellulose ether and water which in the prescribed amount does not harmfully affect the structure and stability of the colloidal composition, a wetting agent, and an aldehyde selected from the group consisting of glyoxal and pyruvic aldehyde.

35 5. A stencil duplicating ink comprising more than 50 percent water as the principal diluent, 3 to 7 percent by weight of a water soluble dye, 2 to 10 percent of hydroxyethyl cellulose, 3 to 25 percent of ethylene glycol, 0.5 to 2.0 percent of a wetting agent, and .25 to 3.0 percent of an aldehyde selected from the group consisting of glyoxal and pyruvic aldehyde.

6. A stencil duplicating ink comprising an aqueous composition consisting essentially of water as the major diluent and carrier, a tinctorial agent, a polyhydric alcohol, a cellulose ether derivative soluble in aqueous media of the type water and dilute alkaline solutions and present in sufficient quantity to provide a body to the ink composition corresponding to a viscosity of 35 to 150 seconds measured by a Stormer viscosimeter operating with a standard cup without a center baffle at 20° C. under a 200 gram load.

55 7. A stencil duplicating ink as claimed in claim 1 in which the cellulose derivative is hydroxyethyl cellulose.

8. A stencil duplicating ink as claimed in claim 1 in which the cellulose derivative is ethyl cellulose having less than one-third of the hydroxyl groups ethylated.

9. A stencil duplicating ink as claimed in claim 1 in which the cellulose derivative is methyl cellulose.

10. A stencil duplicating ink as claimed in claim 3 in which the cellulose ether is hydroxyethyl cellulose.

11. A stencil duplicating ink as claimed in claim 3 in which the cellulose ether is methyl cellulose.

12. A stencil duplicating ink as claimed in claim 3 in which the polyhydroxy alcohol is ethylene glycol.

13. A stencil duplicating ink as claimed in claim 3 in which the polyhydroxy alcohol is diethylene glycol.

14. A stencil duplicating ink as claimed in claim

4 in which the aldehyde is present in an amount ranging from 1 part aldehyde to 2-10 parts by weight cellulose ether.

15. A stencil duplicating ink as claimed in claim 4 in which the aldehyde is present in an amount ranging from 0.25-7.0 percent by weight.

16. A stencil duplicating ink as claimed in claim 4 in which the cellulose ether is hydroxyethyl cellulose and the aldehyde is present in an amount ranging from 0.25-3.0 percent by weight.

17. A stencil duplicating ink as claimed in claim 4 in which the tinctorial agent is a water soluble dye.

18. A stencil duplicating ink as claimed in claim 4 in which the low aliphatic polyhydroxy alcohol is diethylene glycol.

19. A stencil duplicating ink as claimed in claim 4 in which the cellulose ether is hydroxyethyl cellulose, the polyhydroxy alcohol is diethylene glycol and the aldehyde is glyoxal.

THOMAS SEAL CHAMBERS.

ROBERT THOMPSON FLORENCE.

## REFERENCES CITED

The following references are of record in the file of this patent:

## UNITED STATES PATENTS

|    | Number    | Name        | Date          |
|----|-----------|-------------|---------------|
| 5  | 1,645,117 | Schladebach | Oct. 11, 1927 |
|    | 1,930,178 | Mizener     | Oct. 10, 1933 |
| 10 | 1,937,105 | Thomsen     | Nov. 28, 1933 |
|    | 2,393,637 | Jones       | Jan. 29, 1946 |

## FOREIGN PATENTS

|    | Number  | Country       | Date          |
|----|---------|---------------|---------------|
| 15 | 481,911 | Great Britain | Mar. 21, 1938 |

## OTHER REFERENCES

20 "American Ink Maker," June 1945, pages 21, 22 and 23.